

## UNITED STATES PATENT OFFICE

HANS FRIEDELAENDER, OF BERLIN, GERMANY

## TREATMENT OF FIBROUS MATERIAL

No Drawing. Application filed April 9, 1928, Serial No. 268,798, and in Germany May 17, 1927.

This invention relates to the treatment of artificial fibrous material for instance artificial silk, including loose fibres adapted for textile purposes and products formed therefrom.

According to the present invention artificial fibrous material (for instance artificial silk) is treated with emulsions of hard waxes to which are added agents adapted to secure the precipitation of the wax upon the fibres.

The invention may be carried into effect in such manner that products are obtained containing only a relatively small proportion of hard waxes in relation to the fibre. The proportion may, for instance, amount to not more than 1 to 10 per cent. of the dry weight of the fibre.

The invention extends, as above indicated, also to the treatment of loose fibres, for instance cotton, linen, silk, wool or artificial silk, adapted to be spun or otherwise employed for textile purposes.

Preferably in accordance with the invention an emulsion of Montan wax is used as the hard wax and with advantage Montan wax which has in order to refine and harden it, been first fused and heated to a temperature of 230 to 250° C. while air is blown therethrough is employed.

Optionally in accordance with the invention the emulsions may contain oils and similar materials singly or in combination one with the other.

In the treatment of artificial fibres the hard waxes may be and are preferably employed in association with known sizing agents for instance resin.

The following particulars are given by way of example to illustrate suitable methods of carrying the invention into effect:

## Example 1

An emulsion being formed from Montan wax hardened and refined by heat treatment and resin in the proportion of 84 parts to 16 parts is used for treatment of artificial silk threads or hanks by dipping same into the emulsion. Alum or aluminium sulphate is added to the artificial fibrous material in order to precipitate the wax and the product

is treated in known manner for the formation of artificial fibrous articles. These may be satined by treatment between hot rollers.

## Example 2

Saponified Montan wax which has been hardened and refined is incorporated in artificial silk fabric by treating same with the watery emulsion and afterwards fixing the Montain wax in the artificial silk by means of a precipitant. The emulsion employed may contain 80 per cent. of hardened Montan wax, 10 per cent. of oil or fat and 10 per cent. of resin.

## Example 3

Artificial silk fibres are treated with an emulsified mixture obtained by emulsifying hard wax and resin in the proportion of 85 of the former to 15 of the latter. Precipitation is then effected by the employment of aluminium sulphate. The further treatment is effected in known manner and the proportions of the additions made amount to about 10 per cent. of the dry weight of the fibre.

Having now described my invention, what I claim as new and desire to secure by Letters Patent is:

1. The process of producing impregnated artificial fibrous materials, which comprises effecting the precipitation in and on the artificial fibre of hard wax.

2. The process of producing impregnated artificial fibrous materials, which comprises effecting the precipitation in and on the artificial fibre of hard wax from an emulsion thereof.

3. The process of producing impregnated artificial fibrous materials which comprises effecting the precipitation in and on pre-formed artificial fibre of hard wax from an emulsion thereof.

4. The process of producing impregnated artificial fibrous materials, which comprises effecting the precipitation in and on artificial silk of hard wax from an emulsion thereof.

5. The process of producing impregnated artificial fibrous material which comprises

effecting the precipitation in and on the fibre of Montan wax.

6. The process of producing impregnated artificial fibrous materials which comprises effecting the precipitation in and on the fibre of hardened Montan wax.

7. The process of producing impregnated artificial fibrous materials which comprises effecting the precipitation in and on the fibre of hardened Montan wax from an emulsion of Montan wax which has been fused and heated to a temperature of 230-250° C., while air is blown therethrough.

8. The process of producing impregnated 15 artificial fibrous materials which comprises effecting the precipitation in and on the fibre of hard wax from an emulsion thereof containing materials adapted to modify the properties of the hard wax.

20 9. The process of producing impregnated artificial fibrous materials which comprises effecting the precipitation in and on the fibre of hard wax from an emulsion thereof containing oil.

25 10. The process of producing impregnated artificial fibrous materials which comprises effecting the precipitation in and on the fibre of hardened Montan wax from an emulsion of Montan wax which has been first fused 30 and heated to a temperature of 230-250° C., while air is blown therethrough, and which contains a proportion of oil.

11. Artificial fibrous material consisting of 35 a cellulose derivative containing hard wax disseminated throughout the substance of the fibre.

12. Artificial fibrous material consisting of 40 a cellulose derivative containing Montan wax disseminated throughout the substance of the fibre.

13. Artificial fibrous material consisting of 45 a cellulose derivative containing hardened Montan wax disseminated throughout the substance of the fibre.

14. Artificial fibrous material consisting of 50 a cellulose derivative containing Montan wax which has been first fused and heated to a temperature of 230-250° C., while air is blown therethrough, disseminated throughout the substance of the fibre.

15. Artificial fibrous material consisting of 55 a cellulose derivative containing hard wax and materials adapted to modify the properties of the hard wax disseminated throughout the substance of the fibre.

16. Artificial fibrous material consisting of 60 a cellulose derivative containing hard wax and oil disseminated throughout the substance of the fibre.

60 In testimony whereof I have signed my name to this specificaition.

HANS FRIEDLAENDER.